

Jan. 5, 1926.

1,568,224

J. KARAFIAT

BEARING METAL

Filed Feb. 1, 1924



Inventor  
J. Karafiat  
By Marko Orel  
Atlys

## UNITED STATES PATENT OFFICE.

JOSEF KARAFIAT, OF SCHWECHAT, NEAR VIENNA, AUSTRIA.

## BEARING METAL.

Application filed February 1, 1924. Serial No. 690,009.

*To all whom it may concern:*

Be it known that I, JOSEF KARAFIAT, a citizen of the Republic of Austria, residing at Schwechat, near Vienna, Austria, have invented certain new and useful Improvements in Bearing Metals, of which the following is a specification.

This invention relates to bearing metals of the ternary system tin-antimony-lead, 10 which metals, although containing less than 60% of tin, have the same strength, hardness, plasticity and sliding qualities as alloys of that kind with a considerably higher proportion of tin.

15 Alloys of said ternary system, showing various compositions, either with or without other additions, are frequently used in practice as bearing metals. Indications as to their qualities and behaviour in practice 20 are scarce and somewhat contradictory. Theoretical research and investigation of the constitution of these ternary alloys has led to the statements given on a triangular diagram by Loebe, ("Metallurgie," vol. 8, 25 page 7). Furthermore Heyn and Bauer (Verhandlungen des Vereins zur Beförderung des Gewerbeleisses 1914, supplement) have made exhaustive studies and tests in order to obtain reliable data as to their 30 physical properties (fusion- and setting-temperature) as well as to their structure in connection with their strength. But a rule for manufacturing good bearing metals by systematically substituting cheaper 35 alloys for the expensive alloys containing a high proportion of tin did not derive from said scientific research.

In the diagram shown on the accompanying drawing, which diagram represents the 40 composition of the said ternary alloys as usually on an equilateral triangular system, a field marked III is to be seen, by which alloys of well determined compositions are graphically defined. This state field III 45 is bordered by the lines  $E_1-C$ ,  $C-E_2$  and by the irregular line  $E_1-E_2$ , which last line, with its extensions reaching to the sides of the diagram also represents the boundary, at which the separation of bimetallic eutec- 50 tic mixtures takes place.

The present invention consists of constituting a new bearing metal by the addition of metals capable of forming solid solutions with tin and lead (excepting thallium) 55 to main alloys of said ternary system of

such composition, as had hitherto never been combined therewith, viz, with the main alloys tin-antimony-lead of the state field bordered within the said wellknown triangular diagram by lines connecting the following 60 corner points: 10% Sn, 10% Sb, 80% Pb;— 55% Sn, 5% Sb, 40% Pb;—50% Sn, 50% Sb, 0% Pb.

As a result of exhaustive experiments and examinations I have found, that exactly at the boundary between the state fields II and III of said diagram a sudden increase of upsetting capability takes place and that this capability reaches its maximum at the boundary between the state 70 fields III and IV, whilst the reduction of hardness also sets in sharply at the boundary between the state fields II and III and terminates at the boundaries between III and IV. Therefrom it resulted, that alloys 75 of the composition according state field III, which contain two eutectics, viz:  $(Pb-\beta)$  and  $(Pb+\alpha)$  and besides them only  $\beta$ -crystals, (see the work of Heyn and Bauer referred to above) are especially 80 adapted as main substance for bearing metals, provided that they can be hardened without becoming brittle. Thereafter it has been found, that this latter effect can be attained by the addition of metals, which— 85 as mercury, bismuth and cadmium—are capable of forming solid solution with tin and lead. By the addition thereof a most marked amelioration of compressive strength and hardness takes place without 90 any diminution of plasticity and tenacity. An exception is thallium, which, although also forming solid solutions, appears to be unfit for the purpose of the present invention. 95

In practice especially the following composition limits are to be considered for the main substance: Tin 20% to 52%, antimony 12% to 20%, lead 28% to 68%. The amount of the hardening additions is 100 chosen between 0.1% and 3%, for which amount preferably that of the lead is to be reduced. By practical tests it has been stated, that by adding 0.1% to 3% of mercury or bismuth the Brinell hardness 105 index of such soft alloys is increased for about 0.3% to 4% and the specific compressive strength by 25 to 150 kilogrammes per square centimeter. Cadmium, in a quantity of 0.1 to 2%, increases the hard- 110

ness by 1.6 to 12° Brinell, and the compressive strength by 90 to 450 kilogrammes per square centimeter, that is to say by about 30% as a maximum. Accordingly, 5 cadmium is the best means for converting the described main substances into bearing metals, as by small additions of cadmium it is possible to improve the hardness and resistance to compressive strain to such an 10 extent that alloys with an average proportion of tin become equal to alloys with a high proportion of tin. Mixtures of bismuth and cadmium can also be used in the 15 sense of the invention within the same composition limits, for producing bearing metals.

The addition of small quantities of copper 20 prevents in the well known manner, by forming grid, any segregation or liquation, and contributes slightly to an increase 25 of hardness and of compressive strength.

*Examples.*

1. An alloy containing 40% tin, 4.2% 25 copper, 16% antimony and 39.8% lead shows a hardness of 25.4° Brinell and a compressive strength of 1,400 kilograms per square centimeter. If one per cent of lead is replaced by cadmium, the hardness will 30 increase to 33.6° Brinell and the resistance to compressive strain to 1,920 kilograms per square centimeter.

2. If in the above alloy the cadmium is 35 replaced by bismuth, the hardness will be 29.5° Brinell and the resistance to compressive strain 1,600 kilograms per square centimeter. An alloy of a similar composition in which, in place of Bismuth, mercury is used, shows a hardness of 30° 40 Brinell and a compressive strength of 1,640 kilograms per square centimeter.

3. An alloy containing 30.0% tin, 3.5% 45 copper, 16.0% antimony and 50.5% lead, shows a hardness of 26° Brinell and a specific compressive strength of 1,440 kilograms. If 1% lead is replaced by 0.5% cadmium and 0.5% bismuth, the hardness will be increased to 30° Brinell, and the

compressive strength to 1,680 kilograms per square centimeter. 50

What I claim is:

1. Bearing metals of the ternary system tin-antimony-lead with an addition of metals capable of forming a solid solution with tin and lead excepting thallium, the 55 said metals being added to main substance alloys of the state field III of the diagram of the said ternary system, the corner points of which state field represent: 10% Sn, 10% Sb, 80% Pb;—55% Sn, 5% Sb, 40% Pb;—50% Sn, 50% Sb, 0% Pb.

2. Bearing metals of the ternary system tin-antimony-lead with an addition of cadmium, this latter metal being added to main substance alloys of the state field III 65 of the diagram of the said ternary system, the corner points of which state field represent: 10% Sn, 10% Sb, 80% Pb;—55% Sn, 5% Sb, 40% Pb;—50% Sn, 50% Sb, 0% Pb.

3. A bearing metal consisting of 20-52% 70 tin, 12-20% antimony and 28-68% lead with substitution of a part of the lead contents by metals which are capable of forming a solid solution with tin and lead, thallium, although capable of forming a 75 solid solution, being excepted from addition.

4. A bearing metal consisting of 20-52% tin, 12-20% antimony and 28-68% lead 80 with substitution of 0.1-5% of the lead contents by metals which are capable of forming a solid solution with tin and lead, thallium, although capable of forming a solid solution, being excepted.

5. A bearing metal consisting of 20-52% 85 tin, 12-20% antimony, 28-68% lead, part of the lead amounting to 0.1-3% being substituted by equal quantities of cadmium.

6. A bearing metal consisting of 20-52% tin, 12-20% antimony, 28-68% lead, part 90 of the lead amounting to 0.1-3% being substituted by equal quantities of a mixture of cadmium and bismuth.

In testimony whereof I have affixed my signature.

JOSEF KARAFIAT.